

Aug. 5, 1958

L. SCHLECHT ET AL

2,846,299

PRODUCTION OF METAL POWDERS

Filed Dec. 29, 1954



INVENTORS:

LEO SCHLECHT  
ERNST OESTREICHER

BY  
Mayall, Johnston, Cook  
& Post  
ATT'YS

1

2,846,299

## PRODUCTION OF METAL POWDERS

Leo Schlecht, Ludwigshafen (Rhine), and Ernst Oestricher, Ludwigshafen (Rhine)-Oppau, Germany, assignors to Badische Anilin- & Soda-Fabrik Aktiengesellschaft, Ludwigshafen (Rhine), Germany

Application December 29, 1954, Serial No. 478,292

Claims priority, application Germany January 5, 1954

11 Claims. (Cl. 75—5)

This invention relates to the production of metal powders with uniform particle size from metal carbonyls.

In the production of metal powders by thermal decomposition of metal carbonyls in a heated free space it is desirable to obtain a metal powder of which the particle size is uniform and which exhibits a minimum of agglomeration of primary particles to secondary, larger agglomerates. Especially in the processing of metal powders, as for example nickel powder, with very low bulk densities to porous accumulator electrodes, the presence of a considerable proportion of coarse spongy agglomerates, in addition to very fine particles, is detrimental to the properties of the electrodes. These agglomerates prevent the formation of a uniform pore width in the electrode, thereby increase the electrical resistance in the interior of the electrode and reduce the capacity constancy of the accumulator.

The spongy agglomerates present in the powder are also troublesome in other purposes of employment, and in some cases this is attributable to the fact that they have a higher carbon and oxygen content than the finer particles of the powder. This difference in the purity of the various particles of powder is a considerable drawback in working up the powder by powder-metallurgical methods, for example in the production of sintered permanent magnets.

We have now found that the formation of such agglomerates in the production of metal powders, in particular nickel, iron or iron-nickel powders for the production of porous electrodes for alkaline accumulators, by thermal decomposition of metal carbonyls in the free space of an externally heated container can be substantially prevented by keeping those surfaces of the wall of the container which do not serve for the supply of the heat necessary for the decomposition, at a temperature which lies at or slightly above the condensation temperature of the metal carbonyl to be decomposed.

The industrial operation of this process is effected in general by a cooling of that part of the decomposer through which the heat necessary for the decomposition is not supplied, and which without cooling would acquire an undesirably high temperature by radiation or heat conduction. In particular the upper part of the decomposer, where the carbonyl is introduced and which is preferably constructed as a conical cover, is cooled by a cooling means, as for example by a cooling jacket or a cooling coil, to that temperature at which a condensation of the introduced metal carbonyl can still not take place but at which on the other hand any considerable decomposition of the metal carbonyl is no longer possible.

As the cooling medium for the said places of the decomposer it is preferable to use water or steam, and the cooling effect can be adjusted to the desired degree by means of the speed of flow of the cooling medium chosen.

The spatial extent of the cooling is preferably of such dimensions that the cooling action extends up to that part of the decomposer which is externally heated. In

2

this way there is obtained a rapid transition from the low temperature produced by cooling to the high decomposer wall temperature effected by the external heating. The shorter this transition from low to high temperature, the better is the reduction in the formation of coarse agglomerates at this point. It is also preferable so as to construct the decomposer and the cooling means that the transition from low to high temperature takes place where the decomposer has the greatest internal width. It is simplest to choose a cylindrical tube as the decomposer, which is provided at the top with a conical lid which is cooled down to the point at which it is mounted on the tube.

The temperature to which cooling is effected is dependent on the boiling point of the metal carbonyl to be decomposed. Generally speaking the cooling is to the greatest possible extent but not to such an extent that a condensation of the metal carbonyl vapor can take place because otherwise liquid carbonyl in the form of drops will fall through the heated free space and thereby contaminate the powder and render it inflammable and moreover cause the formation of coarse flocculent metal particles. In the decomposition of undiluted iron carbonyl, it is suitable in general to maintain a temperature of about 110° C. in the neighbourhood of the entry of the carbonyl into the decomposer, and this can be effected by using as cooling medium a current of steam of corresponding temperature. In the case of undiluted nickel carbonyl vapor it is preferable to cool to a temperature lying immediately above the boiling point of the nickel carbonyl, for example to 60° C. to 80° C. When working with carbonyl vapor which is diluted with gases, as for example ammonia or carbon monoxide, the temperature necessary according to this invention may lie lower than the boiling temperature of the carbonyl in question because the condensation of the carbonyl vapor takes place only at lower temperatures corresponding to the vapor tension which is reduced by the presence of the diluent gases.

If it is desired to produce a specially light nickel powder, it is advantageous to raise the temperature of the decomposer wall which adjoins the cooled surface to such an extent that this temperature lies at least 270° C. higher than the temperature in the middle of the free space.

In rarer cases it may be necessary to carry out a heating instead of the above-described cooling, namely when the decomposer wall has a temperature which lies below the condensation temperature of the carbonyl. Such spots having too low a temperature can occur in the decomposer when they are too far away from the heat source. By heating these spots to just above the condensation temperature of the carbonyl, the formation of coarse agglomerates can be precluded also in such cases.

The regulation of temperature according to this invention is advantageous irrespective of whether the decomposition of the metal carbonyl is carried out at atmospheric, reduced or increased pressure and with or without dilution with gases or vapors.

Especially when it is desired to produce metal powder with a very low bulk density, there is obtained by the present process a considerable simplification and a considerable increase in the yield of uniformly composed light powder which is very well suited for the production of porous electrodes for alkaline accumulators which are to have a practically invariable capacity.

A further advantage of the process according to this invention lies in the fact that the decomposer provided with cooling can be operated for a long time without interruption whereas without the said cooling the operational time is much shorter and, especially when light

powder is produced, the decomposer becomes clogged in a shorter time and must consequently be shut off and cleaned out.

The following example will further illustrate this invention but the invention is not restricted to this example. The example is given with reference to the accompanying drawing which is a diagrammatic sectional elevation of a carbonyl decomposer.

*Example*

Into container A, of which the upper part is heated by a heating jacket B to an internal temperature of about 230° C., vaporous nickel carbonyl is led continuously from a vaporizer C through a pipe D. The carbonyl vapor enters at the middle of a conical, double-walled lid E which closes the top of the container A. Water at a temperature of 60° C. enters the hollow space of the lid E through inlets F and F<sub>1</sub> and leaves through an outlet G at a temperature of 80° C. In the same way the lower part of the container A is also preferably kept at a temperature between 60° C. and 80° C., an inlet F<sub>2</sub> and an outlet G<sub>1</sub> for the supply and withdrawal of water being provided. Hot gases at a temperature of 550° C. are introduced through a pipe H into the heating jacket B in such a quantity that a temperature of about 220° C. in the central part of the container A is maintained. The heating gas leaves the jacket B through an outlet J. The nickel powder formed by the decomposition of the carbonyl and collecting in the lower part of the container A is removed periodically by means of a sluice K. The carbon monoxide formed by the decomposition leaves the container A through a pipe L and is freed in the usual way by a filter device M from the residual nickel powder which is removed from the filter device through a pipe N.

The particles of the resulting nickel powder, which has a carbon content of 0.09%, are, in spite of the low bulk density of 0.5 kilogram per litre, so small and free from agglomerates that upon sieving through a sieve with 16900 meshes per square centimetre practically no residue remains.

On the contrary by operating in the same decomposer without the above mentioned cooling of the lid, it is true that a nickel powder with the same bulk density is obtained, but it contains large agglomerates of up to 3 millimetres which have a carbon content of 0.21% as compared with a carbon content of about 0.10% in the finer particles. When this nickel powder is sieved, only 75% passes through a sieve with 16900 meshes per square centimetre. If the large agglomerates are removed by mechanical comminution, the yield of fine particles can be increased from 75% to 95%, but the bulk density is thereby increased to 0.8 kilogram per litre and the carbon content of the powder which has passed through the sieve is also increased from 0.10 to 0.15%. This sieved nickel powder has therefore become heavier and less pure and is therefore less suited for use for many purposes, in particular for powder-metallurgical purposes, as for example for the production of porous electrodes.

The process according to the present invention thus not only gives considerably better yields of a more uniform powder without coarse agglomerates, but also a powder with lower bulk density and higher purity than the decomposition of carbonyl without such a temperature regulation.

What we claim is:

1. In a process for the production of a metal powder by thermal decomposition of a metal carbonyl in the free space of a container having the heat of decomposition applied externally through the walls thereof, the improvement which comprises maintaining the inner wall surfaces of the container not utilized for supplying heat for decomposition at a temperature in the vicinity of but above the condensation temperature of the metal carbonyl.

2. In a process for the production of nickel powder by thermal decomposition of nickel carbonyl in the free space of a container having the heat of decomposition applied externally through the walls thereof, the improvement which comprises maintaining the inner wall surfaces of the container not utilized for supplying heat for decomposition at a temperature in the vicinity of but above the condensation temperature of the nickel carbonyl.

10 3. In a process for the production of iron powder by thermal decomposition of iron carbonyl in the free space of a container having the heat of decomposition applied externally through the walls thereof, the improvement which comprises maintaining the inner wall surfaces of the container not utilized for supplying heat for decomposition at a temperature in the vicinity of but above the condensation temperature of the iron carbonyl.

4. In a process for the production of nickel-iron powder by thermal decomposition of a mixture of nickel carbonyl and iron carbonyl in the free space of a container having the heat of decomposition applied externally through the walls thereof, the improvement which comprises maintaining the inner wall surfaces of the container not utilized for supplying heat for decomposition at a temperature in the vicinity of but above the condensation temperature of the mixture of nickel carbonyl and iron carbonyl.

20 5. In a process for the production of nickel powder by thermal decomposition of nickel carbonyl in the free space of a container having the heat of decomposition applied externally through the walls thereof, the improvement which comprises maintaining the inner wall surfaces of the container not utilized for supplying heat for decomposition at a temperature of 60° C. to 80° C.

30 6. In a process for the production of iron powder by thermal decomposition of iron carbonyl in the free space of a container having the heat of decomposition applied externally through the walls thereof, the improvement which comprises maintaining the inner wall surfaces of the container not utilized for supplying heat for decomposition at a temperature of about 110° C.

40 7. In a process for the production of nickel powder by thermal decomposition of nickel carbonyl in the free space of a container having the heat of decomposition applied externally through the walls thereof, the improvement which comprises maintaining the inner wall surfaces utilized for supplying heat for decomposition at a temperature of at least 270° C. higher than that temperature in the middle of the free space, and maintaining the adjacent inner wall surfaces of the container not utilized for supplying heat for decomposition at a temperature of 60° C. to 80° C.

45 8. In an apparatus for the production of a metal powder by thermal decomposition of a metal carbonyl, said apparatus being of the type having a closed elongated container, an inlet for carbonyl vapor, an outlet for metal powder formed in the decomposition, an outlet for carbon monoxide formed in the decomposition, and means for externally applying heat through a portion of the walls of the container to supply the heat of decomposition; the improvement in combination with said apparatus which comprises means for maintaining the inner wall surfaces of the container not utilized for supplying heat for decomposition at a temperature in the vicinity of but above the condensation temperature of the metal carbonyl.

50 9. In an apparatus for the production of a metal powder by thermal decomposition of a metal carbonyl, said apparatus being of the type having a vertically-arranged elongated container including a bottom and side walls, a cover enclosing the container at its upper end, an inlet for carbonyl vapor in the cover, an outlet at the bottom of the container for metal powder formed in the decomposition, an outlet near the bottom of the container for carbon monoxide formed in the decomposition, and means for externally applying heat through at least a portion

of said side walls of the container to supply the heat of decomposition; the improvement in combination with said apparatus which comprises cooling means in said cover for maintaining the inner wall surface of said cover at a temperature in the vicinity of but above the condensation temperature of the metal carbonyl.

10. An apparatus as defined in claim 9 wherein the inner wall surfaces forming a lower portion of the container in the vicinity of the outlets for metal powder and carbon monoxide and not utilized for supplying heat for decomposition are also provided with cooling means for maintaining said inner wall surfaces at a temperature in the vicinity of but above the condensation temperature of the metal carbonyl.

11. An apparatus as defined in claim 9 wherein the 15 cover is a hollow cone having its base adjacent to the side

walls of the container through which the heat of decomposition is applied externally and its apex provided with an opening for the introduction of carbonyl vapor, said hollow cone formed with an outer wall spaced from an inner wall for circulation of a cooling medium between said outer wall and said inner wall.

References Cited in the file of this patent

UNITED STATES PATENTS

|    |           |                       |               |
|----|-----------|-----------------------|---------------|
| 10 | 1,759,659 | Mittasch et al. ----- | Nov. 20, 1930 |
|    | 1,836,732 | Schlecht et al. ----- | Dec. 15, 1931 |

FOREIGN PATENTS

|    |         |                     |               |
|----|---------|---------------------|---------------|
| 15 | 300,691 | Great Britain ----- | Nov. 19, 1928 |
|    | 542,783 | Germany -----       | Jan. 28, 1932 |